

July 16, 1940.

A. JOHNSON ET AL.

**2,207,985**

## MANUFACTURE OF GAS

Filed May 24, 1937



INVENTORS  
ALFRED JOHNSON  
MORRIS M. BRANDEGEE  
BY

*Kenneth J. White*  
ATTORNEY

## UNITED STATES PATENT OFFICE

2,207,985

## MANUFACTURE OF GAS

Alfred Johnson, Summit, and Morris M. Brandegee, Plainfield, N. J., assignors to Combustion Utilities Corporation, New York, N. Y., a corporation of Maine

Application May 24, 1937, Serial No. 144,432

3 Claims. (Cl. 202—23)

This invention relates to the manufacture of combustible gas, and more particularly concerns an improved method of converting petroleum oils into combustible gas of combustion characteristics generally adapted for use in industrial and domestic heating.

Methods heretofore suggested for converting the gas oil and fuel oil fractions of petroleum oil into a fuel gas have not generally been very efficient. One reason for this is that such proposed methods have usually involved a single stage oil cracking operation which yields a gas of relatively low calorific value and gravity, along with considerable production of free carbon, and some heavy petroleum tar and pitch of little value.

The primary object of the present invention is to provide an improved and economically efficient process by which heavy petroleum oil distillates and residual oils may be converted to a fuel gas with a minimum economic loss through conversion to free carbon and unsaleable heavy tar.

Another object of the present invention is to provide improved operating cycles, either continuous or intermittent, whereby existing gas retort benches may be operated efficiently and economically for converting petroleum oils into saleable domestic fuel gas and light oil by-products.

Another object of the present invention is to provide improved operating cycles for existing coal gas retort benches whereby the production capacity of such apparatus may be considerably increased at a minimum cost by simultaneous production of oil gas, coal gas and/or water gas therein without adverse effect on quality of the resulting gaseous, liquid and solid products.

40 A feature of the invention resides in an improved two-stage method whereby petroleum gas oil and fuel oil fractions can be efficiently and economically converted into high yields of marketable light oil and fuel gas products.

45 Petroleum oils, i. e., gas oil and heavy fuel oil fractions, can be cracked by the first low temperature vapor-phase cracking stage of the present process (operating in the temperature range 1100°—1700° F. at atmospheric pressure) to produce a rich gas carrying 87%—18% by weight of the oil used of polymer tar vapors. The tar which is recovered by condensation and scrubbing is a valuable low gravity tar sometimes containing as much as 10%—60% of light oils belonging to the benzene toluene and xylene series.

5 After stripping this tar from the gas the gas has a heating value of 900—1600 B. t. u. per cu. ft., and must be reformed to produce a gas having combustion characteristics more nearly resembling coal gas or water gas or whatever type of gas is finally desired. For producing a final gas of relatively high B. t. u. (for example 1000 B. t. u.) only part of the rich gas produced in the 1st stage need be reformed—after which the 10 balance of the rich gas is admixed with the reformed gas.

15 Another feature of the invention resides in an improved continuous process for simultaneously carbonizing coal and generating both oil gas and coal gas having similar combustion characteristics in a multiple retort coal gas generating unit by an operating cycle which insures segregation of coal-tar and oil-tar by-products, and recovery of an oil tar having a large content 20 of benzol and toluol.

25 With the above and other objects and features in view, the invention consists of the improved method of generating combustible gas which is hereinafter described and more particularly defined by the accompanying claims.

30 In the drawing forming a part hereof there have been illustrated preferred apparatus arrangements adapted for practicing the process of the present invention.

35 The drawing is a view in vertical side elevation, with parts broken away and parts in longitudinal section, showing a horizontal gas retort bench having associated therewith oil and gas injection nozzles and an oil gas purifying and reforming circuit of the type contemplated by the present process.

40 In the drawing the retort bench therein shown embodies a plurality of horizontal gas retorts 110, 110a, having refractory walls 112 surrounded by heating flues 114. Each retort has at its forward end a removable door 116 through which a charge of coal may be introduced to the retort for carbonization, and also through which the completed coke may be discharged. Heat for 45 carbonizing the retort charge is developed by combustion of fuel gas in the flues 114, and is transmitted to the charge by conduction through the walls 112. Gas which is produced in the upper retort 110 during the carbonization of the charge is removed through an off-take pipe 118 which is ported out in the top of the retort adjacent the door 116. This off-take conducts the 50 gas into a hydraulic main 120 through which the gas is carried to purifying equipment and thence to a holder (not shown).

The gas which is produced in retort 110a is removed through an off-take pipe 121 into a gas cooler and interchanger 122, and thence to a tar scrubber 123. From the scrubber 123 purified gas is returned by an exhauster pump 124 through interchanger 122 and pipe 125 to a gas injector 126 which is mounted in the rear wall of retort 110 in position to project an atomized gas-steam mixture into the retort. This rich 10 gas may be forced through a light oil recovery plant by exhauster 124 and circuit 129 prior to its return through cooler 122 to retort 110.

A steam-oil atomizer 127 is mounted horizontally in the rear wall of retort 110a in position 15 to project an atomized oil-steam mixture into the retort. The atomizer 127 is shown as mounted centrally at the cool end of a high temperature refractory tube 128 having its hot end ported out in the retort and extending rearwardly through the back wall of the retort. Oil is conducted to the mixing throat of burner 127 from an oil preheating coil 128, by a valved feed pipe 130. Steam is supplied to the inlet end of the burner 127 from a pipe 132. Provision is 25 made for supplying air and steam to the gas burner 126 through valved pipes 134 and 136, respectively.

The gas retorts can be operated on a continuous or substantially continuous cycle, because 30 heat for their operation is derived by continuous combustion of gas in the flues surrounding the retort walls. While only two retorts have been illustrated, the cycle is designed for application to a bench of several retorts operating on alternate charging and discharging periods.

Coal, preferably bituminous coking coal, is first charged to one or more retorts indicated by the numerical designation 110 to approximately the full depth of the retort, after which the charging doors are closed and heat is applied to the retort by circulation of burning gaseous fuel through the heating flues 114 which surround the walls of the retort. After heating the charges of coal in the retorts 110 for a period of from 45 one to six hours, the top and peripheral portions of the charge in one retort 110 will have been raised in temperature to above 1700° F., with formation of a thin layer of coke. Carbonization of a charge of coal in a retort proceeds from 50 the periphery inwardly at a rate which is substantially inversely proportional to the square of the thickness of the charge. Consequently a retort charge which may require from 12 to 18 hours for complete coking, will develop a layer of coke 2 to 3 inches in depth in its outer periphery within a period of from one to six hours.

After heating the charge of coal in retort 110 for a period of say one to three hours, a second retort 110a is charged with a full charge of previously formed coke, and heat is applied to the charge in retort 110a by circulation of burning gases through the heating flue surrounding this retort, the charging cycles and heating of retorts 110 and 110a being timed so that when 65 a charge undergoing carbonization in retort 110 has been stabilized in the temperature range 1700° F.-2200° F., the temperature of the charge of coke in retort 110a should be substantially simultaneously stabilized at a temperature in the 70 range 1100° F.-1700° F.

At the time the coal and coke charges in retorts 110 and 110a, respectively, have been brought to the above indicated stabilized temperatures, atomized petroleum oil (atomized fuel 75 oil or gas oil) is introduced into the hot coke

charge in retort 110a through the oil atomizer 127. Steam is usually employed for atomizing the oil. The oil is preferably preheated before introduction into the retort 110a by passing it through preheating coil 128 in the waste gas flue 5 which serves for conducting hot flue gases away from the retort setting.

While continuing application of heat to the coke charge in retort 110a by circulation of heating gases through the heating flues 114, the atomized oil or atomized mixture of oil and steam is injected longitudinally into the retort and through the retort charge. It is desirable that introduction of oil, or oil and steam, into the charge in retort 110a shall only take place when 10 the temperature of the retort charge lies in the range 1100° F.-1700° F., and preferably in the range 1300° F.-1500° F. Likewise it is desirable that the introduction of rich gas to the retort charge 110 shall not begin until the temperature 15 of the retort charge in 110 shall have been stabilized in the temperature range 1700° F.-2200° F. During the short time that the atomized oil or oil-steam mixture remains in contact with the charge of coke in retort 110a the oil is cracked 20 forming a rich oil gas of 2100-950 B. t. u./cu. ft. The gas thus produced exits from the retort through off-take pipe 121 and is cooled by passing it through the heat interchanger 122. The rich 25 gas which exits from the retort carries a small amount of oil carbon and as much as 87% by weight of the oil of tar vapors, in suspension. From the interchanger 122 the partially cooled 30 gas enters the base of the scrubber 123, in which the gas intimately contacts a counter-current 35 stream of cold liquid scrubbing medium, preferably water. During the passage of the gas through the length of the scrubber 123 all tar vapors carried by the gas are condensed and scrubbed out of the gas, and the gas is then carried by a return pipe 125 back through an exhauster 124 to the heat interchanger 122 where in it absorbs preheat by heat interchange with the hot gas entering the interchanger from retort 110a. From the interchanger 122 the cleaned 40 and purified rich gas is forced through the gas-steam mixer 126 into and through retort 110, in which a charge of coal is being carbonized. The mixture of devaporized rich oil gas and steam which is introduced into retort 110 enters an 45 atmosphere of coal gas which is continuously being liberated from the charge in the retort as the coal therein undergoes carbonization.

The coal gas which is evolved in retort 110 normally has an average calorific value of 550 55 B. t. u. per cu. ft. and a mean specific gravity of about .50 based on a specific gravity of one for air. By varying the rates of introduction of oil gas and steam through the mixer 126 into the retort 110, and by varying the temperatures 60 obtaining in the retorts 110a and 110 within the temperature range specified, the resulting mixture of reformed oil gas and coal gas can be adjusted as to heating value and specific gravity within the ranges 450-800 B. t. u. per cu. ft. and 65 .40 and .65 gravity. The resulting mixture of coal gas and oil gas may have substantially the same combustion characteristics as coal gas, so that by the present method a retort setting can have its gas producing capacity increased as 70 much as 50% without any substantial increase in plant investment. Furthermore this increase in capacity can be accomplished without any substantial increase in operating cost, because the tar and light oil by-products which are 75

recovered from a by-product tar have a saleable value which substantially pays for the fuel oil which is used in producing the oil gas.

As previously indicated, experience has shown that the optimum yield of saleable liquid by-product and of a suitable rich oil gas adapted for reforming, is secured when the retort 110a is operated at a temperature in the range 1100°-1700° F. and preferably in the range 1300° F.-1500° F. When operating the retort within the above specified temperature range the oil-steam mixture which is introduced to the retort charge, and the oil gas-water gas product thereof, is passed through the retort charge from end to end at a rate such that the atomized oil and resulting cracked oil gas is exposed to the temperatures obtained within the retort for a period of only about 0.25-1.5 seconds.

It will be understood that the retort 110a can be operated as an oil cracking zone without having therein a charge of coke. However, more efficient heat transfer and better cracking is obtained when employing a charge of coke or of small sized ceramic brick in the retort 110a. Retort temperatures below 1700° F. in retort 110a are necessary particularly when employing a coke charge therein, in order to reduce to a minimum the production of unsaleable heavy tar and free carbon. Likewise oil gas may be reformed in retort 110 when the retort is empty or filled with fully carbonized coke or refractory, on a straight two-stage reform oil gas cycle. The carbon resulting from the cracking of oil may be reacted with steam.

When steam is introduced with the oil into retort 110a the proportion of steam to oil is preferably maintained within the limits  $\frac{1}{10}$  to  $\frac{5}{10}$  lb. of steam per lb. of oil. The rate of introduction of oil, or oil-steam mixture, to the retort charge, is also preferably regulated to produce a rich oil gas having a calorific value in the range 950-2100 B. t. u. per cu. ft., while holding the temperature in the retort 110a in the range 1100°-1700° F. In the same way the rate of introduction of oil gas for reforming into the retort 110 is also preferably regulated, as is also the rate of introduction of any steam or air along with the oil gas, so as to produce a reformed gas normally having substantially the combustion characteristics of coal gas, while holding the temperature within the retort 110 within the range 1700° F.-2200° F.

The process, whether conducted on an intermittent or continuous cycle, has two phases, which may be characterized as a rich gas make and a lean gas make. During the rich gas making phase, the principal operation is one of vapor-phase oil cracking and polymerization at relatively moderate temperatures (1100° F.-1700° F.) and usually in the presence of some steam or water gas, to yield a rich gas product of high heating value along with light oils and tar under conditions producing a minimum of free carbon residue. During this first phase steam is not employed during the make in excess of 0.1-0.5 lb. per pound of oil. By stripping the tar and valuable light oil vapors from the rich gas product produced in the first phase of the process—before practicing the second phase during which the stripped high B. t. u. gas product is reformed to a lean make gas—a valuable liquid by-product is recovered and at the same time the gas that is to be reformed in the second phase is stripped of the constituents which are the principal source of the large free carbon waste which is encountered whenever an attempt is made to crack such

oils in one stage operation into a final lean gas product. After the removal of this tar the rich make gas from the first phase can be reformed in the second phase at a higher temperature (1700° F.-2200° F.) by gas phase cracking reactions carried out in an atmosphere of steam, water gas and/or coal gas, substantially without the formation of any free carbon.

To further illustrate the advantages of the process the following table is given which shows the effect of cracking temperature during the first phase of cracking on products recovered from two typical oils:

Cracking results of first stage of cracking when using gas oil, are shown below—

| Temperature cracking                                 | 1100° F. | 1300° F.            | 1500° F. | 1700° F.                        |
|------------------------------------------------------|----------|---------------------|----------|---------------------------------|
| Recoverable light oil pound per pound oil            | .085     | .120                | .100     | .068                            |
| Free carbon produced pound per pound oil             |          | Trace               | .105     | .355                            |
| Liquid tar produced pound per pound oil              | .780     | .400                | .255     | .110 25                         |
| Total light oil, carbon and tar; pound per pound oil | .865     | .520                | .460     | .533                            |
| Percent free carbon in tar (no screen)               |          | .10                 | 29.2     | Above 50% with free deposit. 30 |
| Percent free carbon in tar (with screen)             |          | .10                 | 5.9      | 32.5                            |
| Cu. ft. scrubbed gas per gallon oil                  | 12.7     | 49.2                | 71.9     | 91.0                            |
| B. t. u. per cu. ft. scrubbed gas                    | 1637     | 1525                | 1220     | 905                             |
| Sp. gravity scrubbed gas                             | .965     | .888                | .68      | .465 35                         |
| B. t. u. in scrubbed gas per gallon of oil cracked   | 20,800   | 74,900              | 87,700   | 82,300                          |
| Time of contact                                      |          | .5 sec. to 1.5 sec. |          |                                 |
| Steam pounds per pound oil                           | 0.06     | 0.10                | 0.25     | 0.50                            |

Fuel oil, topped crude or residuum oil may be cracked to oil gas over this preferred low temperature cracking range with good results. The distinguishing difference over use of gas oil being the production of more tar and free carbon and slightly lower gas yields. The calorific value and gravity of the gas over this range of cracking is essentially the same as that secured from gas oil. The following table shows results secured from a 16.5° A. P. I. Bunker C oil containing 10% Conradson carbon.

| Temperature of cracking                              | 1100° F. | 1300° F.            | 1500° F. | 1700° F.                               |
|------------------------------------------------------|----------|---------------------|----------|----------------------------------------|
| Recoverable light oil pound per pound oil            | .064     | .090                | .075     | .051                                   |
| Free carbon produced pound per pound oil             | .100     | .100                | .179     | .366                                   |
| Liquid tar produced pound per pound oil              | .735     | .450                | .341     | .232                                   |
| Total light oil, carbon and tar; pound per pound oil | .899     | .640                | .595     | .649                                   |
| Percent free carbon in tar (no screen)               | 12.0     | 18.7                | 34.5     | Above 50% with free carbon deposit. 65 |
| Percent free carbon in tar (with screen)             | 2.0      | 3.2                 | 7.4      | 19.2                                   |
| B. t. u. in scrubbed gas per gallon oil              | 17,900   | 64,700              | 75,600   | 71,000                                 |
| Time in contact                                      |          | .5 sec. to 1.5 sec. |          |                                        |
| Steam-lbs. per lb. of oil                            | 0.10     | 0.15                | 0.30     | 0.60                                   |

The above cracking results for the first stage of oil cracking for gas and fuel oils over the low cracking temperature range 1100° F.-1700° F. are

obtained when the oil feed and steam rate is that substantially as shown. With higher rates the cracking temperature required to give the same results is slightly greater, although within practical limits the temperature and rates given are productive of best results.

Referring to the above tables it will be seen that as the cracking temperature is increased less recoverable liquid tar is produced, and that the formation of free carbon starts at a temperature slightly below 1300° F., with a rather rapid increase in quantity at temperature in excess of 1500° F. The free carbon yield in the temperature range of 1500° F. to 1700° F. is within practical operating limits for fair operating results, but gives some deposit difficulties with free carbon and stiff heavy tar in the cooling system. It will further be noted that an optimum light oil and thermal hydrocarbon gas recovery occurs in the temperature range of 1300°-1500° F., and that while the tar yield within this range is less than that below 1300° F. the quality is unimpaired with excessive free carbon, as the quantity of the latter, even though not screened out as with coke or refractories in a retort, is not excessive.

We have also noted that an optimum production of toluene, benzol, and xylene occurs over the cracking temperature range of 1300°-1500° F. Below this range the light oil, while aromatic, contains a large per cent of low boiling point paraffin oils, while above this temperature range at 1500 to 1700° F. an optimum yield of benzene occurs, with a rather rapid decline in the toluene yield.

Above 1700° F. the quantity of the light oil fractions falls rapidly. The liquid tar yield is low, free carbon in large quantities appears, and the hydrocarbon thermal yield of gas produced falls.

Having described our invention, what we claim as new is :

1. The process of converting a petroleum fuel oil into fuel gas of predetermined calorific value and specific gravity together with a valuable liquid by-product which comprises, vaporizing and cracking a flowing stream of the oil while admixed with .05-0.3 lb. of steam per lb. of oil at a temperature in the range 1300°-1500° F., and at substantially atmospheric pressure, controlling the rate of passage of the oil steam mixture through the reaction zone to limit the time of exposure of the reaction mixture to the temperatures indicated within a period of  $\frac{1}{2}$ - $1\frac{1}{2}$  seconds, cooling the gaseous reaction products and separating tar and condensable hydrocarbon liquids therefrom, and reheating the resultant fixed gas and flowing it in contact with incan-

descent solid carbonaceous fuel at a temperature of 1700° F.-2200° F. in the presence of sufficient steam to adjust the calorific value and gravity.

2. The process of converting a petroleum fuel oil into a valuable liquid by-product and fuel gas, which comprises atomizing a continuously flowing stream of said fuel oil with 10%-50% by weight of steam and projecting the atomized oil and steam into and rapidly through a bed of hot coke while applying heat thereto in amounts sufficient to maintain the coke bed at oil cracking temperatures in the range 1100° F.-1700° F., simultaneously carbonizing coal in a zone separate from the oil cracking zone, cooling the gaseous products of the cracking reaction and separating therefrom condensable liquid hydrocarbon products, preheating the resulting fixed hydrocarbon gas by heat interchange with the gaseous products of the cracking reaction, and flowing a stream of the gas in admixture with steam continuously through the coal carbonizing zone while applying heat from an external source to the coal and coke charge in amount sufficient to drive off coal gas and to simultaneously reform the oil gas at a temperature in the range 1700° F.-2200° F., to produce a mixture of coal gas, water and oil gas having substantially the combustion characteristics of coal gas.

3. A process of coking coal and manufacturing gas which comprises transmitting heat to a stationary charge of coking coal in a retort and thereby raising the temperature of a portion of the charge above that at which coke is formed and coal gas is liberated, after the body of coal in the retort has been partly converted to coke and the temperature has been stabilized in the range 1700° F.-2200° F., passing an atomized stream of oil through a separate oil vaporizing and cracking zone maintained at a temperature of 1100° F.-1700° F., cooling the cracked oil gas and separating condensable liquid hydrocarbon products therefrom, reheating the tar free gas thereby produced, flowing the gas through the incandescent coke in the retort in admixture with steam while continuing application of heat to the coke in the retort in amounts sufficient to maintain the temperature therein in the range 1700° F.-2200° F., and completing the coking operation while adjusting the time of contact of the oil gas and steam with the coke, and the proportions of oil gas and steam, to produce a reformed oil gas having substantially the combustion characteristics of coal gas, and discharging coke and gas separately from the retort.

ALFRED JOHNSON.  
MORRIS M. BRANDEGEE.